# EUROPEAN PATENT SPECIFICATION

(11) **EP 4 204 636 B1**
(45) Date of publication and mention of the grant of the patent: **20.11.2024**
(21) Application number: 21939586.0
(22) Date of filing: 09.11.2021
(51) Int. Cl.: E04B 2/18, E04C 2/06, E04C 5/02

(54) **ELASTIC REINFORCED COMPOSITE FOR FORMING DIVERSE STRUCTURAL SYSTEMS AND ITS APPLICATION IN MONOLITHIC SANDWICH MATERIAL COMPOSITE**
ELASTISCHES, VERSTÄRKTES VERBUNDMATERIAL ZUR HERSTELLUNG VERSCHIEDENER STRUKTURSYSTEME UND SEINE ANWENDUNG IN MONOLITHISCHEM SANDWICHMATERIALVERBUND
COMPOSITE RENFORCÉ ÉLASTIQUE POUR FORMER DIVERS SYSTÈMES STRUCTURELS ET SON APPLICATION DANS UN COMPOSITE DE MATÉRIAU SANDWICH MONOLITHIQUE

(43) Date of publication of application: 05.07.2023
(73) Proprietor: FLEXCRETE TECHNOLOGY LIMITED, Hong Kong (HK)
(72) Inventor: WONG, Chi Kuen, Tai Kok Tsui, Kowloon (HK); YAU, Yee Sun Calvin, Yuen Long, New Territories (HK)
(74) Representative: Marks & Clerk LLP
(86) International application number: PCT/CN2021/129526
(87) International publication number: WO 2023/082040

(56) References cited:
- WO-A1-2008/035057
- WO-A1-87/04208
- CN-A- 101 979 798
- CN-A- 105 839 818
- CN-A- 110 424 605
- CN-A- 110 616 840
- CN-A- 111 827 147
- CN-A- 113 309 266
- CN-U- 202 596 028
- CN-U- 206 360 399
- CN-U- 210 177 770
- EA-B1- 037 166
- KR-B1- 102 265 607
- US-A1- 2005 210 767
- US-A1- 2009 120 025
- US-A1- 2012 066 994

## Description

### FIELD OF THE INVENTION

This invention relates broadly to an innovative form of Reinforced Cementitious Composite material system having a new interlocking structured rebar network combined with an infiltrated heterogeneous blend hydraulic material in lieu of the ribbed solid metal rebar being widely used in construction industries currently for forming concrete structural elements. As will become apparent, this invention allow the realization of Novel Elastic Reinforced Cementitious Composite characterized with high mechanical bond performance by using interlocking hydraulic material matrix dowel approach and high deformation/ductility capacity by using anti-buckling features of triangular perforated tubular rebar structure lacing with multi-layer perforated metallic plates.

### Prior Art Reinforced Cementitious Composite Technologies

Publications and applications of Reinforced Concrete Composite Technologies are well-known art in construction industry and the merit of it is the ribbed steel rebar providing the concrete structure with tensile strength and complementing the compressive strength of the concrete. However, the steel reinforcing ribbed rebar cage can distort or buckle extensively even restrained by confinement rebar system during high dynamic lateral load, such as earthquake.

With reference to Figures 1, 2a and 2b a typical ribbed solid and/or hollow rebar with different polygonal sectional shapes are shown to demonstrate the typical state of art approach for bonding and anchoring rebar with hydraulic binder matrix material by ribs distributed over the circumference of the core of the solid and/or hollow rod to form structural concrete elements. However the buckling of rebar rod during high dynamic lateral load is still an unresolved and recognized drawback of mono-solid/hollow rebar that result principally due to its low Moment-of-Inertia, Ineffective anchorage mechanism, shear lag size-effect and large elastic modulus mismatch in-between rebar and surrounding cementitious matrix. In a more particular sense, the novel perforated tubular monolithic architected rebar together with the infiltrated normal strength high elastic modulus hydraulic binder matrix which is proposed by the present invention, while retaining all of the important advantages offered by conventional, solid, composite rebar, both significantly, correctively, addresses the mono-solid/hollow rebar limitations and elastic modulus mismatch problem just mentioned, and concurrently introduces new mechanism in rebar matrix interface bonding and reinforcement lap splicing.

In construction industry the technology based on using multiple layers steel mesh as welded solid bar reinforcement network for forming concrete products is generally named Ferrocement laminate Figure 3c and the best known high performance product is DUCON. However its main application is in jointless flooring overlay and concrete reinstatement. Alternative improvement on state of art Ferrocement laminate is also highly desirable.

It is also known that state of the art high performance thin sandwich composite panel system for example steel-concrete-steel (DSC) hybrid panel Figures 3a and 3b is typically composed of dual steel plates as reinforcing skin and sandwiched with Portland cement matrix by using welded steel stud as shear connector. However, welding fatigue problem is one of the major drawback that occur frequently in thin steel plate sandwich composite during service lifetime. Beside the wide adoption of DSC in the construction market is very limited due to the fire proofing requirement of the outermost double skin metal sheets and the prescribed special welding steps for installing the steel shear stud plus the fatigue problem.

Document EA 037.166 B1 discloses an elastic reinforced cementitious composite being made up of elongate perforated tubular metallic material reinforcement with triangular sectional confinement topology configured by three continuous parallel aligned interconnected solid rod-like portion located at triangular apexes respectively as longitudinal reinforcing phase, multiple perforated mid-span shell bandage portion as anchorage phase, and infiltrated heterogeneous blend high elastic modulus hydraulic binder material as matrix phase; wherein the novel perforated tubular reinforcement bar being an extruded closed-shaped metallic material having a triangular sectional topology to maximize the moment-of-inertia of the said reinforcement bar structure; the elongate continuous solid apex corners of the triangular sectional topology reinforcement bar being designated as reinforcing phase to maximize the rigidity of the said reinforcement bar structure; the perforated mid-span shell bandage portion of the triangular sectional topology being designated as anchorage phase with the periodically arranged endless cellular confinement hoops to maximize the matrix dowel interlocking and confinement action of the said reinforcement bar structure; the profile-shaped anchorage end-cap heads maximizing the anchorage capacity and shortening the embedment length requirement of the said reinforcement bar structure; and the infiltrated high elastic modulus ternary blend hydraulic binder matrix material stiffening-up the anti-buckling capacity of the said reinforcement bar structure.

Thus, there is still a need in the art for reinforced laminate structure materials that can be utilized within current design code for structural application, while eliminating the above mentioned limitations in particular cement-based reinforced laminate structures, with large failure toughness and low hydration heat during curing.

### Key Problems in Current Reinforced Cementitious Composite Material Development

Architectural and civil engineering structures, such as buildings, bridges, etc., generally employ a reinforced concrete structure. In a reinforced concrete structure, steel reinforcing in the form of ribbed solid rebar is embedded in cast concrete. The steel reinforcing provides the concrete structure with tensile strength and complements the compressive strength of the concrete. However the steel reinforcing bar/cage can distort or twist causing unnecessary deflection of the resulting reinforced concrete structure. Meanwhile, with the imposition of strict wind and earthquake resistant design, reinforced concrete design specifications regarding confinement transverse reinforcing bar details have been made and widely applied to cater for higher ductility performance of the reinforced concrete structure. Current state of the art reinforced cementitious composite materials are limited in arranging cross-tie loop bar as confinement reinforcement in combination with mono-solid/hollow rebar and the buckling issue of solid rebar under seismic load still remain unresolved. Notably, as the diameter of traditional, solid, composite rebar increases, the "shear-lag" problem leads to the combined negative effects of non-proportional core-strength increasing and losing core-area efficiency in terms of strength and load handling. Other common practice to improve ductility of reinforced concrete is adding metal fiber to prevent the concrete from cracking but only limited result can be achieved unless dose with very high fiber content. Such major drawback regarding traditional solid steel rebar is principally due to its "buckling"- limitations which, importantly, are now successfully addressed by the features of the present, "perforated-tubular" two-main-component apex solid/mid-span shell, composite rebar invention, shortly to be more fully disclosed.

Very interestingly, the apparatus employed by the invention to make the proposed new perforated tubular rebar structure, and the associated making methodology, collaboratively contribute significantly to the manufacturability of the prevent invention that enhance its utility in this field.

Another aspect of the present invention, the development of elastic reinforced monolithic laminate composite concept base on three-dimensional tension interlocked confinement reinforcement cage network. By tailoring the non-slip topological interlocking mechanism, debonding failure due to interfacial crack propagation between the reinforcing phase and matrix phase of reinforced cementitious composite could be alleviated and segmentation of infiltrated cementitious continuous matrix by the confinement reinforcement cage network into hard and soft phases further translate their individual structural properties into advanced composite material.

The invented three-dimensional tension interlocked confinement reinforcement cage network utilize the full capacity of the continuous reinforcing phase from inner to outer uniformly. Unlike the traditional friction force between conventional rebar and matrix, interfacial bonding is not the main action for the transfer of forces in this novel elastic reinforced composite system. Instead the fully rigid composite action is invoked by the interlocked and distributed anchorage network force transfer mechanism between the three-dimensional reinforcement phase and the infiltrated high elastic modulus matrix binder material.

More elaborations about these new features and advantages are presented now immediately below in the respective summary descriptions as well as later on in the detailed description of the invention.

### SUMMARY OF INVENTION

### Novel Reinforced Cementitious Composite Systemic Features

From a systemic perspective, the invention may be described as a composite-rebar network material system expressible as including (a) an elongate, triangular perforated tubular rebar structure, and a defined-function collar-sleeve fitting joined to that perforated triangular tubular rebar element, (b) a perforated cellular transverse reinforcing metal plate for arranging a plurality of perforated triangular tubular rebar forming reinforcing bar networks, and (c) a low hydration heat high elastic modulus infiltrated cementitious matrix embedding the perforated triangular tubular rebar element/networks.

The present invention, in addition to the systemic perspective of the above, further propose a new composite-material anchorage bonding mechanism in lieu of ribs bonding as a result of the robust dowel interlocking mechanism in-between triangular perforated tubular rebar network and high elastic modulus infiltrated matrix together with the laterally spaced perforated cellular reinforcing plate in lieu of transverse rebar.

Another feature of the present invention is to provide a method of constructing a high deformation capacity and ductility structural system having a new reinforcing bar topology configuration which enables better bond strength and reduction of development length through the distributed perforated hole arrangement and apex material-volume usage.

### Tubular, Composite, Apex Solid/Mid-span Shell Rebar Structure

According to a preferred and best-mode embodiment of the invention, what is proposed, from a structural, product point of view, is an elongate, hot-extruded tubular metallic material rebar composite structure formed unitarily and homogenously, having a long axis, and including, (a) three interconnected continuous apex solid rod portions as reinforcing phase, (b) multiple perforated mid-span shell bandage portions as anchorage phase along the length of the rebar, (c) profiled head portions as splice connection phase and (d) hot-extruded tubular metallic collar-sleeve as contact lapping phase. Preferably, the hot-extruded tubular rebar and collar-sleeve are triangularly cylindrical, and the perforated mid-span shell structure possessing longitudinally patterning square dowel holes. Created integrally with and as a part homogeneously of the preferred, triangular perforated tubular rebar with the configuration of the apex solid/mid-span shell bandage combination which centrally defines the rebar confinement structure of the present invention, collaborate to offer significant performance advantages over all known solid rebar structures, including unique anti-buckling load managing, maximum material-moment of inertia distribution to counteract the "shear-lag" problem confronts traditional solid rebar-usage designers in "size effect" dilemma and high interface mechanical bonding/anchorage mechanism to effectively retaining good internal coherence with infiltrated cementitious matrix material.

Importantly, the seamless monolithic anti-buckling bandage nodal zone existing between the continuous apex solid reinforcing phase and the mid-span shell which has resulted from a single hot extrusion manufacturing procedure hold the endless hoop confinement capability for restraining matrix dilating borne force and directing them effectively into the long, linear axially extending, tension-capable apex corner rods present in the rebar structure.

In the proposed, preferred-embodiment rebar structure, the dimension of the continuous apex solid portions (8mm-16mm) are sized effectively to achieve sufficient failure toughness and at the same time minimize the lap-length parameter, where, in the design standards, it is considered 40 times of bar diameter.

### Collar-Sleeve Splice Connector and Triangular Reinforcing Rebar Networks

Another key feature of the present invention is that it offers, for useful and innovative employment, snugly inserted connections by means of a perforated triangular tubular collar-sleeve over both profiled dual-headed ends of two perforated triangular tubular rebars of the same outside dimension.

The collar-sleeve, per se, in the rebar structure of the invention is independently expressible as being a jacketing-structure possessing similar physical form and properties as the rebar structure with an offset-dimensionality extend structure. This innovative connection model facilitates and reduces the assembly cost of the invented rebar structure, is describable as an integral-form of contact lapping splice sleeve associated with interlocked dowel keys.

Another extremely interesting feature of the perforated triangular tubular rebar structure of the present invention is that, rebar networks structure can be effectively assembled involving simple insertion of multi-layer perforated cellular metal plates as transverse reinforcement. Not only is this feature of the invention by itself interesting, the cellular transverse reinforcing metal plate, also employed as embedded "internal endless loop" reinforcing inclusions, dramatically avoid the dilation phenomenon of infiltrated cementitious matrix typically occurred during earthquake action. This innovative insertion assembly model can measurably improve the efficiency of construction and shorten the construction period via incorporation of modularized rebar network cage for on-site assembly.

### Synergistic Infiltrated Matrix Filler

The present invention, as mentioned above, also proposes infiltrated low hydration heat high elastic modulus cementitous matrix forming interlocking dowel networks for interface bonding and anchorage mechanism inside the novel reinforced composite material. Such high elastic modulus matrix play an important role in the deformation and ductility performance of the present invention in structural application. Put another way, being an infiltrated inorganic hydraulic binder based material, both the low yield stress rheological mix properties of the fresh paste and high elastic modulus properties of the hardened paste are mandatory in the proposed, preferred-embodiment matrix structure.

As in the state of art practice, one will note that, with conventional cementitious matrix mixing approach, the attainment of high elastic modulus concrete will invoke an upgraded change in the elastic modulus of aggregate employed and or using concrete compressive strength grade above 100MPa. However, with concrete compressive strength grade above 80MPa, large amount of binder hydration heat release during hardening is a major issue that cause concrete internal cracking unless appropriate cooling procedure is properly executed drying curing and even fibre reinforcement is mandatory in building regulation to prevent expose cracking under fire.

For reasons not completely understood and which have surprised us, the fact that the unique ternary composition binder containing ultra-fine Ultrafine Ground granulated blast furnace slag (UFGGBS) at (15%-35%), and more preferably at (25%-35%), by weight of the total binder with water/binder ratio at 0.28-0.32 of the present invention provide superior elastic modulus enhancement characteristics in the range of 40GPa-45GPa for normal grade 60MPa compressive strength concrete without using ultra-high strength concrete approach, herein so-called "decoupling-effect". This novel low heat ternary composition cementitious binder together with the organic osmotic spacer dispersant hereafter named "G.Seed" may have significant improvement in the C-A-S-H gel morphology and bond density due a large portion of Ultra-fine Slag induced aluminate silicate bridging molecules interface strengthening effect. Thereby the hardened matrix closely resemble metallic alloy matrix in term of the modulus strengthening approach by using in-situ seeding template to control the gel grain morphology and size of the basic gel building blocks of C-A-S-H so that they can self-assemble into microstructures with far greater bond packing density together with the shifting of amorphous gel state towards ordered crystalline gel state after matrix solidification.

In the proposed, preferred-embodiment novel reinforced composite material, the high elastic modulus infiltrated cementitious matrix hereafter named "ModulusCEM" is formed of air-cured hydraulic active binder which contain Portland cement (OPC), Ground granulated blast furnace slag (GGBS) and Ultrafine Ground granulated blast furnace slag (UFGGBS),organic osmotic spacer, fine aggregate, coarse aggregate, water and organic dispersing agents. Importantly, the preferred infiltrated cementitious matrix takes the form of an optimized packing bond density paste dispersed combinatorially with small molecular organic osmotic-spacer co-dispersant present in the fresh mixed matrix for imparting dense packing filling effect at low water/binder-ratio.

Preferably after hardening, the interfacing transition zone exiting between paste and aggregate, according to preference, takes the form of a dense thin layer which has resulted from the pozzolanic reaction of ultra-fine active hydraulic mineral filler is essential to the novel reinforced composite for distributing crack control and obtaining high durability.

### Architected Monolithic Sandwich Structure

The present invention, as mentioned above, also proposes novel elastic reinforced sandwich laminate composite material system. In its broadest aspect, this elastic reinforced laminate composite "Architected Cellular Layers material" can be characterized as a "Triangular Interlocked Material (TIM)" based on a combination of ternary composition binder containing ultra-fine Ultrafine Ground granulated blast furnace slag "normal strength-high elastic modulus matrix" and a three-dimensional reinforcement cage confinement network derived from assemblages of aligned multiple layers perforated iso-grid patterned metal plates which is internally tension interlocked with a plurality of inter-fitted apex solid triangular hollow rebars in at least one dimension. The apex solid triangular hollow rebars acting as transverse reinforcement system within the multi-layer monolithic sandwich composite counteract separation through matrix dowel anchorage mechanism and give a strong tension interlocking action, even under conditions of heavy destruction where matrix might fail.

The invention is now ascertained by creating an innovative "Triangular Interlocked Material - TIM" structured-structures laminate design and pre-determined topological configurations approach which are characterized by what is stated in the independent claims. The preferred embodiments of the invention are disclosed in the independent claims. In particular, the "Triangular Interlocked Material (TIM)" system are derived from assemblages of unit cells, where each of the unit cells has a solid triangular cylindrical core geometry configuration with the top and bottom faces bounded by endless cellular confinement hoop based on a triangular motif ordered inside the slender-beam architected two-dimensional perforated grid plate. The unit cell's dimension parameters has a profound control effect in developing the dowel properties of unit cell through confinement action attributed from the non-slip topological interlocking action in-between the reinforcing structure phase and matrix phase. This obviate the traditional composite reinforcing limitation based on bond stresses force transfer to alloy the full tensile strength of the reinforcing phase. As an effective structural materials, the periodically replicated cellular cylindrical solid dowels with well-controlled "interlocking parameter" triangle geometry hereafter named as "Triangular Interlocked Material (TIM)" confer the Architected Cellular Layers Material system with tunable mechanisms, precise structural properties and functionalities. Thus "TIM" could be assigned as the control representative volume element (RVE) and induce the mechanical properties of the invented composite. The "Triangular Interlocked Material (TIM)" shape factor has the highest intrinsic efficiency ratio defined as the ratio of bonded lateral surface area of the cylindrical material to its cross sectional area for a given equivalent height and unit mass of the matrix material. As such, for the same cross-sectional area, the triangular interlocked material (TIM) is around 30% more effective than a circular shape in developing surface adhesive force and significantly improve the shear strain capacity for a given displacement demand.

Unlike the traditional conception of multi-layer sandwich structures, this invented novel elastic reinforced sandwich laminate composite material system is a novel class of multi-layer sandwich composite material having multi-materials structured-structures hybridization strategy being focused on pre-determined topological configurations inclusive of cellular, layers and segmented structures to constitute ordered phases with differing connectivities, optimally serving specific engineering purpose. In particular, this invention relates to mono- or multi- layer sandwich composite where the stiffness mismatch limitation between the reinforcing and matrix phase is intentionally controlled for fabricating novel elastic reinforced monolithic sandwich composite of incredibly high strength, high flexural stiffness, high ductility, high deformation capacity and high tolerance of local mechanical damage couples with minimum mass. This innovative and realizable thin composite panel can be conceptualized as a highly modified form of infiltrated type laminate sandwich composite without using adhesive or welding technique for binding the dual outer layer sheets with the core. To substitute the adhesive or welding method, a plurality of apex solid perforated hollow rebar which function as tension interlocking connectors and spacers are inserted as bridging anchor rods which firmly binding the dual sandwiched outer layer composite panel sheets with the sandwiched inner layer composite panel core and thereon deliberately generate a fully rigid thin laminate sandwich composite component or element for general structural applications.

### Apparatus for Implementing Novel Rebar and Perforated Plate -Making Methodology

The present invention, as mentioned above, also proposes special apparatus for carrying out the methodology of the invention in order to produce the rebar structure and perforated metal plate of the invention.

The proposed apparatus, progressing therein, and therealong, from the upstream region toward the downstream region, includes (a) a triangular profile mandrel having a long axis which is substantially coincident with the rebar-formation axis, (b) an elongate, hollow pultrusion-die disposed operatively adjacent the extrusion region, having a long axis which is substantially coincident with the rebar-formation axis, circumsurrrounding the mandrel, (c) plural heaters distributed in spaced relation with respect to one another along the rebar-forming axis and disposed in operative adjacency relative to and association with the pultrusion mold die, and (d) a power-driven pusher moving a preheated solid metal rod at a rate relative to the pultrusion-die.

Additionally included in the apparatus of the invention is a fibre-laser tube cutting machine having a rotatable clamp holder coincident with the rebar-forming axis and operable to form pre-defined hole cutting in a manner distributed along the length of the mid-span shell of the rebar structure.

These and various other features and advantages of, and offered, the present invention will become more fully apparent as the detailed description of it below is read in conjunction with the accompanying drawings and the appended claims.

### BRIEF DESCRIPTION OF THE DRAWINGS

Figure 1 shows typical prior art rib-rebar structure with solid or hollow configuration;
Figures 2a and 2b show typical prior art rib-rebar cage assembly, splice lapping and reinforced concrete column-beam joint using headed rebar or bent-shape rebar arrangement;
Figures 3a, 3b and 3c show typical prior art typical sandwich panel and ferroconcrete;
Figure 4 shows three dimensional views of proposed novel rebar structure network including monolithic triangular perforated tubular longitudinal rebar and perforated transverse reinforcement plate;
Figure 5a is a flow chart showing design of novel reinforced cementitious composite;
Figure 5b is a diagram showing strength range of novel reinforced cementitious composite;
Figure 6a shows configuration of novel reinforced cementitious composite;
Figure 6b shows self-standing state triangular bar network with mutual insertion of multi-layered perforated cellular plates;
Figure 7 are schematic views showing collar-sleeve join connection arrangement;
Figure 8a is a Multi-Layered View of Architected Cellular Layers Material;
Figure 8b is a TIM View of the Architected Cellular Layers Material of Figure 8a;
Figure 8c is a Matrix View of the Architected Cellular Layers Material of Figure 8a;
Figure 8d is a perforated Plate View of the Architected Cellular Layers Material of Figure 8a;
Figures 8e and 8f are TIM Hoop Section View and hard-soft matrix domain view of the Architected Cellular Layers Material of Figure 8a;
Figure 9 is a flowchart of Architected Cellular Layers Material design and fabrication;
Figure 10 shows a Unit-cell As Dowel Network of Architected Cellular Layers Material;
Figure 11 is a Hard and Soft Matrix Phase Deformation Diagram;
Figure 12 shows testing of multi-layer monolithic sandwich composite showing stretch-bending fully rigidity composite action;
Figure13a shows ternary binder particle size composition matrix;
Figure 13b are tables showing proposed high elastic modulus binder matrix mix design and properties in fresh and hardened state;
Figure 13c are tables showing cementitious composite design flow chart;
Figure 13d are tables showing test result of proposed high elastic modulus binder matrix in hardened state;
Figure 14 are photos showing hot extrusion production of monolithic triangular tubular rebar with apex solid comers;
Figure 15 are schematic views showing application of novel reinforced cementitious composite for column-beam assembly and modular unit fabrication;
Figures 16a and 16b are photos of finished Panel and Volumetric Prefabricated Concrete Component using Novel Elastic Reinforced Composite Technology;
Figure 17a and 17b are 3D Model showing using Novel Elastic Reinforced Composite Technology in building design and manufacturing.

### BEST MODE FOR CARRYING OUT THE INVENTION

Turing now to the drawings, and referring first of all to Figure 6a, inclusive, indicated generally at (10) the novel reinforced cementitious composite material is an elongate, linear, composite material constructed in accordance with a preferred and best-mode embodiment of the present invention. Triangular Perforated Tubular Rebar (20) which has a long axis seen at Figure 4 includes continuous solid apex reinforcing phase portion (21), mid-span shell anchorage phase portion (22), profiled end-cap head anchorage phase portion (24), and perforated cellular dowel hole interlocking phase portion (23). Embedded integrally and homogenously with the Rebar (20) is the Infiltrated high elastic modulus matrix (40) which has a dense mass form after hardened disposed along the length of the Rebar (20), includes Array of matrix dowels (42), Confined matrix (41) within Rebar envelope and Unconfined matrix (43). Accordingly, the perforated tubular composite rebar structure proposed by the present invention, plays the evident role of furnishing excellent, longitudinal anti-buckling stability for the rebar structure when it is in place within a body of infiltrated high elastic modulus matrix. Illustrated at Figure 4, an array of Dowel holes (23), along the rebar mid-span shell, is the main interlocking interface for developing matrix bond and anchorage strength in lieu of state of art typical rebar ribs along the surface of rod and bent hook arrangement at end of solid rod bar. Collectively the main continuous solid apex corners (21), perforated mid-span shells (22), along with the dual-end-cap head (24) formed by hot extrusion and fiber-laser cutting, are referred to herein collectively as a perforated- tubular-rebar structure (20).

As was mentioned above, perforated tubular rebar is a hot extrusion structure and it allow required elongation characteristics as traditional solid steel rob rebar under tension force applied. The formation of homogeneous apex solid corners and mid-span shell structure includes a mass of a suitable metallic ingot, preferably low carbon steel, and hot extruded through a mold die oriented in perpendicular to the rebar longitudinal axis. Those skilled in the art will readily understand that the various dimensions of the component portions making up the rebar structure (20) may have a relatively wide range of satisfactorily usable and different dimensions, depending upon the particular application for that structure.

Dimensional changes in the rebar component also play a role, of course, in the design load-handling capability of that structure. The fact that the structure, as a whole is a perforated tubular structure, result in substantial elimination of what was described above as the so-called "rebar size shear lag issue" which characterizes conventional large diameter solid rebar. Accordingly, relatively large overall rebar structures are thus producible and usable for high load-handling requirements without the diminution of capability that characterizes large solid-cross-section rebar.

Looking specifically at Figure 4, the reinforcing phase (21) is strategically located at the apex comer of an equilateral triangular sectional geometry to maximize the Moment-Of-Inertia of the rebar structure (20). This configuration of three continuous apex interconnected elongated solid-like rods (21) will eliminate the "shear lag" dilemma that an increase in rebar diameter size to achieve hoped-for greater reinforcing strength. By periodically confining the triangular sectional with seamless, homogenous, and endless hoop bandage stiffeners that run circumferentially as nodes or bulkheads, referred herein as a bandage structure, it further guard against Brazier buckling of proposed reinforcing bar structure for enhancing deformation capacity during seismic action.

In principle, anything which stiffens a tubular rod to buckling will also increase its resistance in bending and so it stronger in compression. Therefore, a quantum jump in strength and ductility of the proposed tubular rebar structure can be realized by providing elaborate structural efficiency in substantially linear, long-axis-tension-carrying-capable reinforcing apex solid, preferably made of metallic material and takes the designated architected form from extrusion formation and fibre laser cutting process.

Especially interesting about this capacity of the bandage rebar structure of the present invention is that such changes in anti-buckling capability may be made without in any way altering the material volume occupied by rebar structure within the infiltrated matrix. In other words, there is provided a striking counter-balance action between rebar anti-buckling handling capability and surrounding matrix dilation during earthquake and lateral force driven.

Directing attention now to Figure 4, by architecting the "Multi-Cellular Matrix Dowel" unit cells (42) along the mid-span shell (23) as anchorage phase, both the bond strength and anchorage development length long-standing issues that have been experienced in conventional steel rib rebar configuration can now successfully addressed by this unique feature of the present invention. Importantly, the intrinsic efficiency in area to volume ratio of "Triangular" sectional shape further maximize the bond existing between the proposed rebar intrinsic angular surface and infiltrated matrix.

This distributed local interlocking mechanism as shown in Figures 4 and 6a, follow the similitude theory in scale change (i.e. Reinforcing Phase + Anchorage Phase + Configuration + Scale) by shifting the design phase of reinforcing component scale to the material scale. Thereby the traditional approach for shortening rebar development length such as using welded anchorage head replacing end hooks can be simplified by a more unified approach through integrated profile shaped end-cap (24).

Describing now the composition of infiltrated high elastic modulus matrix "ModulusCEM" (40), and looking at the overall composition as shown in Figures 13a and 13b, it includes hydraulic mineral binder "G.Seed" (47) with ternary blend cementitious materials (45), fine aggregate, coarse aggregate, organic dispersant, organic osmotic-spacer co-dispersant (46) and water.

Considering aspects of the behaviour of the infiltrated high elastic modulus matrix of the present invention, in addition to those general performance features which are the requirements of cementitious composite such as concrete, are the low yield stress flowing during fresh state and high bond density after hardening in order to obtain high elastic modulus characteristics for the infiltrated inorganic binder matrix.

Focusing for a moment on the hydraulic mineral binder composition, the inclusion of large amount of ultra-fine active mineral filler (UFGGBS), have been purposely to develop high bond density with aggregate, under the organic osmotic-spacer co-dispersant effect, for achieving high elastic modulus paste. This leads to a major improvement over the prior art methodology in using volcanic aggregate which cause alkaline silica reaction. Another state of the art alternative is to employ ultra high strength concrete with compressive strength above 80 MPa, however addition of organic fibre is required for explosive crack control.

As an important performance factor for deformation control of the novel reinforced cementitious composite, the proposed active mineral filler bond density compositional methodology involves what we refer to as a modified form of strength-elastic modulus decoupling effect which differs from aggregate modulus upgrading practice commonly adopted in strength-elastic modulus coupling mix design as depicted in Figures 13c.

The high elastic modulus hydraulic binder, as has also already been mentioned and test result shown in Figure 13d may take on a particular compositional mix based on ternary blend cementitious material (45) includes Ordinary portland cement (OPC), Fine ground granulated blast furnace slag (GGBS), and Ultra-fine ground granulated blast furnace slag (UFGGBS) associated with Organic osmotic-spacer co-dispersant (46) can be made from the following "GSeed" recipe:
(a) 50-60 vol % of Portland cement with average grain size 30µm;
(b) 25-30 vol % of UFGGBS with average grain size 5 µm;
(c) 15-20 vol % of GGBS with average grain size 20µm;
(d) Water/binder ratio in-between 0.28 - 0.32;
(e) 0.5-2 vol % of organic osmotic-spacer co-dispersant.

The novel "ModulusCEM" composite performance after 28 days normal curing are shown in Figure 13d test result table. It clearly demonstrate the high effectiveness of C-A-S-H binder gel layers interfacing strengthening strategy to improve cementitious composite elastic modulus without employing ultra high strength concrete design approach.

Preferably, as shown in Figure 5, the perforated tubular rebar structure of the present invention employ triangular geometry cross-section shape which endowed with highest bending- torsion rigidity. Beside it has largest surface area/volume ratio for maximizing matrix infiltration penetration and flow rate. More specifically, the triangular sectional geometry of the preferred embodiment effectively results in an extremely strong and robust mechanical coupling action between the rebar structure and infiltrated matrix - a bond which also plays a very important role for stiffening the continuous apex corner reinforcing phase against buckling force.

Regarding the triangular perforated tubular rebar splice connection mechanisms, unlike the traditional solid rebar typical lapping arrangement, the collar-sleeve insertion proposed by the present invention as illustrated in Figure 7 is a radical way of integrating splice sleeve and contact lapping methodology commonly adopted separately in state of art solid rebar splice connection.

Perforated tubular collar-sleeve is one of the very unique contributions of the present invention in that it cooperates in a very special way to align perforated tubular rebars coaxially for emulating non-splice continuous rebar tensile load bearing capacity.

As an important aspect of this just-described connection methodology, the proposed snugly insertion methodology including the steps of (a) minimizing the lapping length parameter of apex solid comer reinforcing phase, (b) matching the outside dimensions and geometry of coaxial rebar structure with inside dimensions and geometry of collar-sleeve, and (c) effecting interlocking bonding mechanism with infiltrated high elastic modulus matrix. Particularly distinguishing this integral connection approach from the state of art approaches is the included presence of the profile dual-end-cap head (24) of the perforated tubular rebar which is anchorage-bearing, and cooperatively, engaged with the collar-sleeve (25).

Moving attention now to yet another, the systemic, facet of the present invention, this facet recognizes the opportunities, furnished by the perforated tubular rebar structure of the invention to construct rebar assembly systemically, as for examples, (a) forming triangular rebar network column cage, (b) forming triangular rebar network beam cage, and (c) forming triangular rebar network foundation cage.

Accordingly, Figures 6a and 6b pictures a multi-layer perforated cellular transverse reinforcement plate (30) sandwiched in-between a plurality of triangular perforated tubular rebar (20) forming composite-cellular rebar cage system. These multi-layered three-dimensional architected cellular composite rebar cage structure, also referred to as confinement-cage components, collaborate with the infiltrated high elastic modulus matrix to offer the high deformation and ductility features of the novel reinforced cementitious composite that take advantage of the invention-proposed anti-buckling perforated tubular rebar structure for resisting both the wind and seismic load which act laterally on the building (70).

Illustrated in Figures 6a and 6b the three-dimensional architected cellular rebar cage composite (50) having at least two perforated metal plate (30) with repeated pattern of triangular endless cellular hoops (31) that are aligned, spaced and parallel with one another being designed matchingly to engage with at least two axially aligned triangular perforated tubular rebar (20) in such a rebar network cage structure thereby compulsory act together as high-stiffness confinement envelop for forming "Interlocked Dowel" unit cells (41) distributed within the novel reinforced cementitious composite element structure. The formed "Interlocked Dowel" unit cells exploit its confinement reinforcement capacity effectively to the maximum yielding level before occurrence of matrix slipping and crushing failure. Hence, confinement is monolithic and consequently the composite rebar cage can establish highest energy absorption capacity to dissipate dynamic forces applied on the novel reinforced cementitious composite element. This ultra-ductile ability indicate that the proposed preferred-embodiment of the invented reinforced composite work together as a whole to obtain higher levels of strength, stiffness and resilience mechanical properties in resisting compressive, wind and seismic load while retaining good internal coherence.

In one preferred embodiment the triangular perforated tubular rebar (20) is fabricated from hot extruded low carbon steel material, herein has an overall length of about 10m-12m and possesses a central, long, axis referred to as rebar-formation axis. Extending in a manner along the apex corner axis are continuous solid rod region of approximately drawn diameter (8mm-25mm) - the dimension which defines the effective sectional area of the reinforcing phase. The associated mid-span shell bandage region has thickness of about (3mm-6mm) and width of about (6mm-12mm) - the dimension which defines the effective sectional area of the anchorage phase. The endless cellular hoop region has area of about

(25mmx25mm - 50mmx50mm) - the dimension which defines the effective sectional area of the interlocking matrix dowel.

In one preferred embodiment of the three-dimensional architected cellular rebar confinement cage composite (50), the multi-layered perforated cellular transverse reinforcing phase (30) has equilateral triangle hoops (31) of length size (40mm-70mm) with small rounded vertices that are spaced to create an isogrid topology patterned rib and node web for achieving the best local confinement effect and the perforated plate has thickness of about (2mm-5mm).

In one preferred embodiment the infiltrated high performance matrix binder material (40) as shown in Figure 13c is a high elastic modulus cementituous binder matrix material with a compressive strength between (60MPa-80MPa) and an elastic modulus above 40GPa to provide the requisite strength, hardness and tough ductile behaviour, and the maximum aggregate size is limited to one quarter of the cellular hoop size for unblocked infiltration.

In an exemplar embodiment, the elastic reinforced composite structure as shown in Figure 8 is an elastic reinforced laminate sandwich composite (10) with a plurality of perforated thin metallic plate (30) engineered with endless cellular equilateral triangle hoops as multi-layer transverse reinforcement network bodies. A global three-dimensional cellular confinement cage network as reinforcing phase are constituted by inter-fitting a plurality of apex solid perforated triangular hollow rebar (20) as shear connectors and tension interlocking multi-layered transverse reinforcement bodies thereby a elastic reinforced high performance thin laminate sandwich composite component can be generated after infiltration of the normal strength high elastic modulus ultrafine matrix (40).

As is hereinafter more fully described, the elastic reinforced laminate sandwich composite (10) as shown in Figures 8, 9, 10, 11 and 12 is a three-dimensional architected cellular layers material composite has at least two perforated metal plate (30) with repeated pattern of endless cellular hoops (31) or (31a) and a group of apex solid perforated triangular hollow metal rebar (20) as tension interlocked reinforcement inserted preferably with staggered configuration arrangement in-between perforated metal plates (30) at defined locations. Under this aligned configuration arrangement, the replicated patterned endless cellular hoops (31) or (31a) of the multi-layered perforated metal plate (30) are reciprocally opposite with respect to each other as illustrated in Figure 8e and thereby compulsory cooperate together as high-stiffness confinement envelop of the "Triangular Interlocked Material (TIM)" unit cells (41&42). The formed "TIM" cells consume its reinforcement capacity to the maximum yielding level before occurrence of high performance matrix slipping and crushing failure. Hence, confinement is monolithic and consequently the multilayer structure reinforcing phase can establish higher energy absorption capacity to dissipate dynamic forces applied on the composite panel. This ultra-ductile ability indicate that the invented composite panel work together as a whole to obtain higher levels of strength, stiffness and resilience mechanical properties in resisting compressive, wind and seismic load.

This exemplar invention is based on an unexpected discovery that uniformly distributed local hoops confinement effect can be synergistically generated in-between the infiltrated high performance matrix binder material core and the integral continuous reinforcing structure phase featured with endless cellular hoop architected by rib and node web reinforcement structure. By purposely inter-fitting a plurality of apex solid perforated triangular hollow tube rebars with functionally graded multiple layers perforated metal plates, a three-dimensional cellular reinforcement cage network phase are formed for distributing endless cellular triangular shaped confinement loops into three-dimensional periodically networked pattern which are systematically spaced. By using these inter-fitting operation, a novel architected material having continuous reinforcing and matrix phases can be fabricated while using conventional constituent material and translating their individual structural properties into advanced composite material performance. This invented Architected Material having Cellular and Layers lattice configurations engineered inside Sandwich hybrid material topology obtain its novel elastic reinforced monolithic composite material properties through tension interlocking reinforcement and matrix dowel anchorage mechanism working synergistically within the continuous matrix phase being partitioned into hard domain and soft domain phases by the configuration of cellular confinement rebar network cage. The hard domain (41 & 42) consist of the unit cells based solid triangular cylindrical core geometry dowel matrix and the soft domain (43) consist of the hexagonal honeycomb cellular core geometry matrix as shown in Figures 8a, 8c, 8d and 8f. This combination of triangular and hexagonal domain configuration of matrix phase will maximize the interface strain gradient density to produce high back-stress work hardening for further enhancing laminate composite ductility during deformation. Thereby optimize the composite material design for strength, stiffness and resilient at minimum mass.

By following the design flowchart as shown in Figures 5a, 5b and 9 the mechanical properties of the present invention can be tailored for the intended application and the method presented above provide a clear advantage in manufacturing structural components by avoiding welding and or adhesive processes but instead allow insertion based methodology for fabricating reinforcement configuration in the final desired geometry.

As shown in Figures 6a and 8, the inter-fitted three-dimensional continuous reinforcing phases (50) are assembled from multiple layers of cellular triangular hoop engineered perforated plate (30) through simple insertion operation permitted by the apex solid perforated hollow rebar (20) derived from the complimentary shape configuration, thereby totally eliminate welding and adhesive procedure currently used in honeycomb sandwich and DSC production. This leads to a major improvement over the prior art manufacturing requirements mandated in the DSC (Double Skin Composite) and honeycomb sandwich composite design. This way the production cost significantly is slashed down and recap the full beneficial potential of simple inter-fitting operation.

Finally the triangular perforated tubular rebar structure, the collar-sleeve connector, and the perforated cellular metal plates components of the invented rebar cage composite (50) as shown in Figure 6b, can be robotically assembled with the advent of computer aided design (CAD) and computer aided manufacture (CAM). Using CAD/CAM the perforation cutting pattern can be design in CAD software. The design can then be used to program for the cutting and milling processes as shown in Figures 14, 17a and 17b. The time and labour savings make it possible to economically produce one of a kind product. With CADCAM high volume and low cost product of the three-dimensional architected cellular rebar cage composite (50) is possible.

Accordingly, as shown in Figures 15, 16a and 16b a plurality of novel reinforced cementitious composite formed structural elements such as columns, beams and laminated panels are arranged to fabricate the prefabricated prefinished building modular components (60) in factory and then deliver to construction site for the on-site assembly of building (70) in the next assembly stage. The above described manufacturing and production process of the invented three-dimensional architected cellular layers material sandwich composite as shown in Figure 12 clearly show that no welding or adhesive glue technique are employed for forming the said composite. It exemplify the easily adoption of the said invention in established prefabrication plants with minor modification on existing equipments and fully demonstrate the broad industrial applicability of the said invention.

Today's industry 4.0 trend dictates that construction sector be creative. This architected cellular layers material approach cherish and absorb well established manufacturing technologies and exploit new composite force transfer mechanism to gain innovative and exciting solution as exemplified in the best mode for carrying out the invention. While the best mode for carrying out the invention has been described in detail, those familiar with the art to which this invention relates will recognize various alternative designs and embodiments for carrying out the invention as defined by the following claims.

## Claims

1. A novel elastic reinforced cementitious composite (10)
being made up of elongate monolithic seamless perforated tubular metallic material reinforcement bar with triangular sectional confinement topology configured by three continuous parallel aligned interconnected solid rod-like portion located at triangular apexes (21) respectively as longitudinal reinforcing phase, multiple perforated mid-span shell bandage portion as anchorage phase, and infiltrated heterogeneous blend high elastic modulus hydraulic binder material as matrix phase, wherein an unique, core-radial, axial-align, distributed mechanical bond anchorage dowel network effected from multi-cellular matrix dowel unit cells (42) synergistically formed unitarily with endless cellular confinement hoops (31) along the perforated mid-span shell during hydraulic binder composite solidification; the novel perforated tubular reinforcement bar (20) being an extruded closed-shaped metallic material having an equilateral triangular sectional topology to maximize the moment-of-inertia of the said reinforcement bar structure;
the elongate continuous solid apex corners (21) of the equilateral triangular sectional topology reinforcement bar being designated as reinforcing phase to maximize the rigidity of the said reinforcement bar structure;
the perforated mid-span shell bandage portion (22) of the equilateral triangular sectional topology being designated as anchorage phase with the periodically arranged endless cellular confinement hoops (31) to maximize the matrix dowel interlocking and confinement action of the said reinforcement bar structure;
the elongate continuous solid apex corners (21) being monolithically connected by the perforated mid-span shell portions (22) of the said reinforcement bar in order to maximize the composite bonding action with the infiltrated matrix thereby eliminating the shear lag effect of traditional thick solid reinforcement bar structure;
the elongate continuous solid apex corners (21) being monolithically connected by the perforated mid-span shell bandage portions to maximize the anti-buckling capacity of the said reinforcement bar structure;
the profile-shaped anchorage end-cap heads (24) maximizing the anchorage capacity and shortening the embedment length requirement of the said reinforcement bar structure;
the infiltrated high elastic modulus ternary blend hydraulic binder matrix (40) material stiffening-up the anti-buckling capacity of the said reinforcement bar structure;
the novel triangular shaped perforated tubular reinforcement bar being engineered with multi-cellular confinement dowel unit cells network (42) as principal matrix interface interlocking bonding mechanism of the said reinforcement rebar structure; and
the novel triangular shaped perforated tubular reinforcement bars being longitudinally assembled to form self-standing state triangular reinforcement bar network by coupling with a plurality of multi-layered metallic plate (30) having triangular shaped perforated receiving holes configured as lateral reinforcement confinement hoop system.

2. The elastic reinforced cementitious composite of claim 1, further **characterized in**:
having a laminate topology;
at least one domain of said elastic reinforced cementitious composite having a three-dimensionally reinforced composite structure comprising a partitioned Ultrafine Ground granulated blast furnace slag based cementitious matrix (A) with a tension interlocked cellular hollow rebar network structure (B) wholly embedded in matrix (A), the matrix system (A) comprising a plurality of in-situ formed triangular cylindrical cellular hard inclusion dowel units phase (C), and a plurality of replicated hexagonal cellular soft units phase (D), the tension interlocked rebar network (B) comprising multi-layered perforated triangular hole patterned plates (E) stacking up in parallel and tension interlocked by a plurality of apex solid perforated triangular hollow rebar bodies (F) in transverse direction;
architecting the triangular shaped tension interlocked reinforcement components dimension, alignment and density for toughness tuning;
architecting the layer volume, thickness and spacing of the parallel stacked iso-grid rib patterned perforated metallic plates for compressive strength, rigidity and ductility tuning; and
architecting the in-situ formed anchorage matrix dowel network confinement topology for shear strength tuning.

3. The elastic reinforced cementitious composite according to claim 1, further **characterized in**:
(a) including "ModulusCEM" having infiltrated heterogeneous blend tuneable high elastic modulus hydraulic binder "G. Seed" matrix material;
(b) said ternary blend hydraulic binder matrix material comprising Portland cement (OPC), Ground granulated blast furnace slag (GGBS) and Ultrafine Ground granulated blast furnace slag (UFGGBS) in associated with polymer co-dispersant as osmotic spacer to synergistically forming fresh matrix material with low yield stress, low viscosity rheological properties while, after hardening, possessing high elastic modulus mechanical properties derived from optimized bond packing density of the said ternary binder;
(c) said ternary blend hydraulic binder matrix material comprising highly effective Co-dispersant agent to enhance ultrafine active mineral filler filling ability of the binder and optimized global packing density with least water-film thickness;
(d) said ternary blend hydraulic binder matrix material having composition at the best performance arranged in proportion as OPC-30µm (50-60%), GGBS-20µm (10-25%), UFGGBS-10µm~5µm (15-35%) by weight of total binder content;
(e) said ternary blend hydraulic binder matrix material with water to binder ratio for the best performance assigned at 0.30-0.33 to achieve self compacting ability during casting stage with flow range in between 650mm-800mm by adjusting fluidizing agent dosage;
(f) said ternary blend hydraulic binder matrix material with binder to aggregate ratio at the best performance designates as 0.30-0.33 to achieve high global packing density; and
(g) said ternary blend hydraulic binder matrix material at the best performance after full curing at 28 days having elastic modulus in the range of 35-45 GPa, and compressive strength in the range of 60-80 MPa.

4. The elastic reinforced cementitious composite of claim 3, further **characterized in that** the ternary blend hydraulic binder matrix material at the best performance after full curing at 28 days has elastic modulus in the range of 40-45 GPa.

5. The elastic reinforced cementitious composite of claim 1, further **characterized in that** the monolithic seamless perforated tubular metallic material reinforcement bar with triangular sectional topology includes:
(a) high anti-buckling capacity developed from the restraining action of the periodically spaced closed form triangular hoop bandage node of the tubular reinforcement bar;
(b) high non-slippage bonding strength through interlocking confinement dowel action between reinforcement bar and concrete matrix;
(c) high mechanical anchorage strength through straight and/or L-shaped profile end-cap to shorten embedment development length;
(d) high confinement capacity endless cellular hoops configured by perforated mid-span shell thickness at least 3-6mm, perforated hole size at least 25-40mm and cross-link bar width at least 6-12mm;
(e) high failure toughness with apex interconnected solid-like rod section diameter in the range of 8-25mm;
(f) high tensile yield steel strength in the range of Steel Grade 275-500; and
(g) high ductility and deformation capacity with elongation percentage at least 20-30%.

6. The elastic reinforced cementitious composite according to claim 1, **characterized in** having self-standing state triangular reinforcement bar network with:
(a) high effective lateral support restraining action effected by the interlocked matting action between a plurality of periodically spaced perforated transverse reinforcement plates and a plurality of elongate perforated longitudinal tubular metallic reinforcement bars;
(b) high shear rigidity perforated transverse reinforcement plates with isogrid rids configuration and equilateral triangular holes for the coupling insertion of the perforated tubular metallic reinforcement bars; and
(c) high failure toughness with perforated lateral reinforcement plates thickness in the range of 3-6mm.

7. The elastic reinforced cementitious composite of claim 1, further **characterized by**:
(a) using triangular sectional topology perforated tubular collar-sleeve connector for splice connections between two co-axial perforated tubular rebars of the same outside dimensions;
(b) using bent-shaped/multi-branched collar-sleeve connector for aligning, orientating multiple splice connection joints among a plurality of perforated tubular rebar;
(c) having perforated tubular collar-sleeve connector inside dimensions equals to outside dimensions of the two co-axial perforated tubular rebars such that snugly insertion connection are reliably formed;
(d) having an integral form of contact lapping and splice sleeve mechanism for making continuous force transfer in-between the continuous solid apex corners of perforated tubular collar sleeve and co-axial perforated tubular rebars; and
(e) using infiltrated cementitious matrix dowel anchorage mechanism for interlocking perforated tubular collar-sleeve and co-axial perforated tubular rebars.

8. The elastic reinforced cementitious composite of claim 1, further **characterized by**:
(a) using hot extrusion metallic tube forming process to achieve high elongation tensile properties;
(b) using fibre laser fabrication process to define high precision perforation dimensional properties associated with minimum heat zone effect (HAE); and
(c) using fibre laser etching process resulting in roughened rebar structure surface texture for enhancing bonding characteristics.

9. The elastic reinforced cementitious composite of claim 1, further **characterized in** being for use as structural components and/or elements in forming in-situ and/or prefabricated reinforced cementitious composite components, and having:
(a) high sectional ductility performance for both axially and/or horizontally load structural components effected by the high stiffness distributed hoops tension action of the periodically spaced perforated transverse metal plate as anti-dilating internal reinforcement;
(b) high deformation capacity for both axially and/or horizontally load structural components effected by the three dimensional architected cellular rebar confinement cage structure, thereby furnishing a unique, and effective, distributed interlocking dowel cell units in the reinforced cementitious composite; and
(c) high seismic response performance for beam-frame structural components effected by the core zone hoops tension reinforcement of the self-standing state triangular reinforcement bar network by providing resistance against diagonal tension due to shear in continuous manner.

10. The elastic reinforced cementitious composite of claim 9, further **characterized in that** said prefabricated reinforced cementitious composite components include column, beam and beam-frame system for erection of buildings and civil structures.

11. The elastic reinforced cementitious composite of claim 2, further **characterized in that** the perforated triangular hole patterned plates (E) is an engineered fine grain material having:
(a) the perforated metal plate formed by hot-rolled low carbon thin metal with high tensile strength being at least 250 MPa and high elongation ductility being at least 20%;
(b) the architected hoop with triangle geometry, preferably equilateral shape to form the periodic grid rib and node web having nearly isotropic property and distributed endless hoop confinement elements;
(c) the architected hoop with lengthwise dimension in between 30mm-70mm with non-blurring and or blurring rim;
(d) the high-stiffness fine grain matrix perforated plate reinforcing phase with plate thickness in-between 2mm-5mm and stacking spacing in-between 30mm-100mm, which is at least 2.5 times the dimension of the maximum aggregate grain size of the infiltrate matrix phase;
(e) the rid web with thickness dimension in-between 5mm-20mm;
(f) the endless triangle motif hoops of the perforated grid plate having an optimum form factor ratio between the total perimeter length of the hoop and maximum aggregate grain size of the matrix phase at least greater than 10; and
(g) the endless triangle motif hoops of the perforated grid plate having hoop size which is at least 2.5 times the dimension of the maximum aggregate grain size of the infiltrate matrix phase.

12. The elastic reinforced cementitious composite of claim 11, further **characterized in that** the architected hoop with lengthwise dimension in between 40mm-60mm with non-blurring and or blurring rim.

13. The elastic reinforced cementitious composite of claim 11, further **characterized in that** the high-stiffness fine grain matrix perforated plate reinforcing phase is with stacking spacing in-between 40mm-60mm.

14. The elastic reinforced cementitious composite of claim 11, further **characterized in that** the rid web with thickness dimension in-between 5mm-15mm.

15. The elastic reinforced cementitious composite of claim 11, further **characterized in that** the endless triangle motif hoops of the perforated grid plate has an optimum form factor ratio between the total perimeter length of the hoop and maximum aggregate grain size of the matrix phase at least greater than 20.

16. The elastic reinforced cementitious composite of claim 2, further **characterized in that** the monolithic three-dimensionally reinforced composite structure is a sandwich topology grouping of a plurality of high stiffness plate shaped matrix embedded with elongated reinforcement components in first, second and third dimensions with minimum mass with:
(a) the high resistance against peeling on bending with larger active connection zone by employing sandwich topology as thin panels assembled in bundles forming composite panels corresponding to a larger moment of inertia;
(b) the minimized stiffness mismatch limitation between the reinforcing and matrix phases; and
(c) the elimination of welding and or adhesive material inside the composite to thereby realize a compact fatigue resistant structure.

17. The elastic reinforced cementitious composite of claim 2 for use as structural element or component, further **characterized in** comprising:
(a) multiple layers metal perforated grid plate elements (E) for interlocking (b);
(b) plurality of perforated hollow metal tubular reinforcing bodies (F) as connectors and spacers generating (c);
(c) interlocking three-dimensional grid cells continuous reinforcing structure phase (B) and stiffened by (d);
(d) infiltration of high performance inorganic cementitious matrix binder material (A) and after hardening synergistically forming (e); and
(e) fully rigid thin mono- or multi- layered architected monolithic laminate shaped sandwich composite structural component or element with high intrinsic strength to weight ratio for general and specialized applications in construction and other industries.

18. The elastic reinforced cementitious composite of claim 2, further **characterized in** having multi-materials structured-structures hybridization strategy with pre-determined topological configurations inclusive of cellular, layers and tubular configured structures to constitute ordered material phases to form mono- and or multi- layer sandwich composite with:
(a) high compressive and tensile strength, high stiffness;
(b) high global ductility and deformation capacity; and
(c) high tolerance of local mechanical damage.

19. The elastic reinforced cementitious composite of claim 2, further **characterized in that** the monolithic three-dimensionally reinforced composite structure is a sandwich topology grouping of a plurality of high stiffness plate shaped matrix embedded with elongated apex solid perforated triangular hollow reinforcement components in first, second and third dimensions with minimum mass with:
(a) the high resistance against peeling on bending with larger active connection zone by employing sandwich topology as thin panels are assembled in bundles forming composite panels corresponding to a larger moment of inertia;
(b) the minimized stiffness mismatch limitation between the reinforcing and matrix phases; and
(c) the elimination of welding and or adhesive material inside the composite to thereby realize a compact fatigue resistant structure.

20. The elastic reinforced cementitious composite of claim 6, further **characterized in** being minimized by having direct overlapping of confinement hoops for transferring force in adjacent plates.

21. The elastic reinforced cementitious composite of claim 11 for use as structural components or elements in manufacturing modular components for adoption of assembly type construction method during on-site operation.

22. The elastic reinforced cementitious composite of claim 21, further **characterized in that** said structural components or elements are composed of mono layer architected cellular laminate wall panels and slab panels, which, after mutually assembling the said modular components on site followed by in-situ infiltration of matrix (A) form a plurality of the elastic reinforced cementitious composite of claim 2.

23. A building for habitation composed of structural components or elements, wherein said structural components are comprised of the elastic reinforced cementitious composite of claim 21 and a plurality of the elastic reinforced cementitious composite of claim 2.

## Patentansprüche

1. Neuartiger elastischer verstärkter Zement-Verbundwerkstoff (10), der aus einem langgestreckten, monolithischen, nahtlosen, perforierten, röhrenförmigen Bewehrungsstab aus metallischem Material mit einer räumlichen Struktur der Einschließung von dreieckigem Querschnitt besteht, die durch Folgendes konfiguriert ist: drei kontinuierliche, parallel ausgerichtete, miteinander verbundene, massive, stangenartige Abschnitte, die sich jeweils an Dreiecksscheitelpunkten (21) befinden, als Längsverstärkungsphase, mehrere perforierte Schalenbandagenabschnitte in Feldmitte als Verankerungsphase, und ein infiltriertes heterogenes gemischtes hydraulisches Bindemittelmaterial mit hohem Elastizitätsmodul als Matrixphase, wobei während der Verfestigung des Verbundwerkstoffs aus hydraulischem Bindemittel ein einzigartiges, kernradiales, axial ausgerichtetes Netzwerk aus Verankerungsdübeln mit verteilter mechanischer Bindung, das durch Dübeleinheitszellen einer mehrzelligen Matrix (42) erzeugt wird, einheitlich mit endlosen zellenförmigen Einschließungsringen (31) entlang der perforierten Schalenmitte synergistisch ausgebildet wird;
wobei der neuartige perforierte röhrenförmige Bewehrungsstab (20) ein extrudiertes metallisches Material von geschlossener Form mit einer räumlichen Struktur ist, deren Querschnitt ein gleichseitiges Dreieck ist, um das Trägheitsmoment der Bewehrungsstab-Struktur zu maximieren;
wobei die langgestreckten, durchgehenden, massiven Scheitelecken (21) des Bewehrungsstabs mit der räumlichen Struktur von gleichseitig dreieckigem Querschnitt als Verstärkungsphasen bezeichnet werden, die dazu dienen, die Steifigkeit der Bewehrungsstab-Struktur zu maximieren;
wobei der perforierte Schalenbandagenabschnitt in Feldmitte (22) der räumlichen Struktur von gleichseitig dreieckigem Querschnitt als Verankerungsphase mit den periodisch angeordneten Ringen der endlosen zellenförmigen Einschließung (31) bezeichnet wird, um die Verflechtungswirkung und die Einschließungswirkung der Bewehrungsstab-Struktur auf die Matrixdübel zu maximieren;
wobei die langgestreckten, durchgehenden, massiven Scheitelecken (21) durch die perforierten Schalenabschnitte in Feldmitte (22) des Bewehrungsstabs monolithisch verbunden sind, um die Verbundbildungswirkung mit der infiltrierten Matrix zu maximieren und dadurch den Scherverzögerungseffekt einer herkömmlichen dicken, massiven Bewehrungsstab-Struktur zu beseitigen;
wobei die langgestreckten, durchgehenden, massiven Scheitelecken (21) durch die perforierten Schalenbandagenabschnitte in Feldmitte monolithisch verbunden sind, um die Knickschutzfähigkeit der Bewehrungsstab-Struktur zu maximieren;
wobei die profilförmigen Verankerung-Endkappenköpfe (24) die Verankerungsfähigkeit maximieren und die erforderliche Einbettungslänge der Bewehrungsstab-Struktur verkürzen;
wobei die Matrix aus dem infiltrierten, aus drei Stoffen gemischten hydraulischen Bindemittelmaterial mit hohem Elastizitätsmodul die Knickschutzfähigkeit der Bewehrungsstab-Struktur versteift;
wobei der neuartige dreieckig geformte, perforierte, röhrenförmige Bewehrungsstab mit einem Netzwerk aus mehrzelligen Einschließungsdübeleinheitszellen (42) als Hauptbindungsmechanismus zur Verflechtung der Matrix-Grenzflächen der Bewehrungsstab-Struktur konstruiert ist; und
wobei die neuartigen dreieckig geformten perforierten röhrenförmigen Bewehrungsstäbe längs zusammengebaut werden, um ein selbststehendes Dreiecksbewehrungsstab-Netzwerk zu bilden, und zwar durch Koppeln mit einer Vielzahl von mehrschichtigen Metallplatten (30) mit dreieckig perforierten Aufnahmelöchern, die als ein Ringsystem zur lateralen Bewehrungseinschließung konfiguriert sind.

2. Elastischer verstärkter Zement-Verbundwerkstoff nach Anspruch 1, ferner **dadurch gekennzeichnet, dass**:
er eine geschichtete räumliche Struktur aufweist;
mindestens eine Domäne des elastisch verstärkten Zement-Verbundwerkstoffs eine dreidimensional verstärkte Verbundwerkstoffstruktur aufweist, die eine unterteilte Hochofenzement-Matrix (A) aus ultrafein gemahlenem Hüttensand mit einer spannungsverflochtenen, zellenförmigen, hohlen Bewehrungsstab-Netzwerkstruktur (B), die vollständig in die Matrix (A) eingebettet ist, umfasst, wobei das Matrixsystem (A) eine Phase (C) aus einer Vielzahl von vor Ort ausgebildeten dreieckigen, zylindrischen, zellenförmigen, harten Einschließungsdübeleinheiten und eine Phase (D) aus einer Vielzahl von replizierten sechseckigen zellenförmigen weichen Einheiten umfasst, wobei das spannungsverflochtene Bewehrungsstab-Netzwerk (B) mehrschichtige perforierte Dreieckslochmusterplatten (E) umfasst, die parallel aufeinandergestapelt und durch eine Vielzahl von an den Scheiteln massiven dreieckigen angeordneten perforierten hohlen Bewehrungsstab-Hohlkörpern (F) in Querrichtung spannungsverflochten sind;
er die dreieckigen spannungsverflochtenen Bewehrungskomponenten in Bezug auf Dimension, Ausrichtung und Dichte zur Abstimmung der Zähigkeit auslegt;
er Schichtvolumen, -dicke und -abständen der parallel gestapelten, mit isogitterförmigen Rippenmustern versehenen perforierten Metallplatten zur Abstimmung von Druckfestigkeit, Steifigkeit und Duktilität auslegt; und
er die räumliche Struktur der Einschließung des vor Ort gebildeten Verankerungsmatrix-Dübelnetzwerks zur Abstimmung der Scherfestigkeit auslegt.

3. Elastischer verstärkter Zement-Verbundwerkstoff nach Anspruch 1, ferner **dadurch gekennzeichnet:**
(a) **dass** er ein "CEM-Modul", der ein hydraulisches Bindemittel-"G.Keim"-Matrixmaterial mit heterogenem infiltriertem Mischungsverhältnis und hohem abstimmbarem Elastizitätsmodul aufweist;
(b) wobei das aus drei Stoffen gemischte Hydraulikbindemittel-Matrixmaterial Portlandzement (OPC), granulierten Hüttensand (GGBS) und ultrafein granulierten Hüttensand (UFGGBS) in Verbindung mit einem polymeren Co-Dispergiermittel als osmotischer Abstandshalter umfasst, um synergistisch ein frisches Matrixmaterial mit rheologischen Eigenschaften von niedriger Fließspannung und niedriger Viskosität auszubilden, während es nach dem Aushärten mechanische Eigenschaften mit hohem Elastizitätsmodul besitzt, die sich aus der optimierten Bindungspackungsdichte des Dreistoff-Bindemittels ergeben;
(c) wobei das aus drei Stoffen gemischte Hydraulikbindemittel-Matrixmaterial ein hochwirksames Co-Dispergiermittel umfasst, um die Füllfähigkeit mit ultrafeinem aktivem mineralischem Füllstoff des Bindemittels und eine optimierte globale Packungsdichte mit geringster Wasserfilmdicke zu verbessern;
(d) wobei das aus drei Stoffen gemischte Hydraulikbindemittel-Matrixmaterial bei den besten Leistungsmerkmalen eine Zusammensetzung aufweist, die in einem solchen Verhältnis angeordnet ist: OPC-30 µm (50-60 %), GGBS-20 µm (10-25 %), UFGGBS-10 µm~5 µm (15-35 %), bezogen auf das Gewicht des gesamten Bindemittelgehalts;
(e) wobei das aus drei Stoffen gemischte Hydraulikbindemittel-Matrixmaterial bei den besten Leistungsmerkmalen ein Wasser-Bindemittel-Verhältnis von 0,30-0,33 aufweist, um eine Selbstverdichtungsfähigkeit während der Gießphase mit einem Fließbereich zwischen 650 mm und 800 mm durch Nachregeln der Dosierung eines Verflüssigungsmittels zu erreichen;
(f) wobei das aus drei Stoffen gemischte Hydraulikbindemittel-Matrixmaterial bei den besten Leistungsmerkmalen ein Bindemittel-Zuschlagstoff-Verhältnis von 0,30-0,33 aufweist, um eine hohe globale Packungsdichte zu erreichen; und
(g) wobei das aus drei Stoffen gemischte Hydraulikbindemittel-Matrixmaterial bei den besten Leistungsmerkmalen nach vollständiger Aushärtung nach 28 Tagen einen Elastizitätsmodul im Bereich von 35-45 GPa und eine Druckfestigkeit im Bereich von 60-80 MPa aufweist.

4. Elastischer verstärkter Zement-Verbundwerkstoff nach Anspruch 3, ferner **dadurch gekennzeichnet, dass** das aus drei Stoffen gemischte Hydraulikbindemittel-Matrixmaterial bei den besten Leistungsmerkmalen nach vollständiger Aushärtung nach 28 Tagen einen Elastizitätsmodul im Bereich von 40-45 GPa aufweist.

5. Elastischer verstärkter Zement-Verbundwerkstoff nach Anspruch 1, ferner **dadurch gekennzeichnet, dass** der monolithische, nahtlose, perforierte, röhrenförmige Bewehrungsstab aus metallischem Material mit einer räumlichen Struktur von dreieckigem Querschnitt einschließt:
(a) hohe Knickfestigkeit, die sich aus der Rückhaltewirkung der periodisch angeordneten, geschlossenen dreieckigen Ringbandagenknoten des röhrenförmigen Bewehrungsstabs ergibt;
(b) eine hohe rutschfeste Verbundfestigkeit durch die Verriegelungswirkung der Einschließungsdübel zwischen Bewehrungsstab und Betonmatrix;
(c) hohe mechanische Verankerungskraft durch eine gerade und/oder L-förmige Profilendkappe, um die Einbettungsentwicklungslänge zu verkürzen;
(d) endlose zellenförmige Ringe mit hoher Umschließungsfähigkeit, die durch eine Dicke der perforierten Schale in Feldmitte von mindestens 3-6 mm, eine Größe des Perforationslochs von mindestens 25-40 mm und eine Breite der Querverbindungsstäbe von mindestens 6-12 mm konfiguriert sind;
(e) hohe Bruchzähigkeit mit einem Durchmesser der an den Scheiteln miteinander verbundenen massiven Stange im Bereich von 8-25 mm;
(f) hohe Stahl-Streckgrenze im Bereich der Stahlsorte 275-500; und
(g) hohe Duktilität und Verformungsfähigkeit mit einem Dehnungsgrad von mindestens 20-30%.

6. Elastischer verstärkter Zement-Verbundwerkstoff nach Anspruch 1, **dadurch gekennzeichnet, dass** er ein selbststehendes Netzwerk aus dreieckigen Bewehrungsstäben aufweist, mit:
(a) hochwirksamer seitlicher Abstützung-Rückhaltewirkung, die durch die ineinandergreifende Mattierung-Wirkung zwischen einer Vielzahl von periodisch angeordneten perforierten Querbewehrungsplatten und einer Vielzahl von langgestreckten perforierten röhrenförmigen metallischen Bewehrungslängsstäben bewirkt wird;
(b) perforierten Querbewehrungsplatten von hoher Schersteifigkeit mit Isogitter-Rippenkonfiguration und gleichseitig dreieckigen Löchern zum koppelnden Einsetzen der perforierten röhrenförmigen metallischen Bewehrungsstäben; und
(c) hoher Bruchzähigkeit mit einer Dicke der perforierten seitlichen Bewehrungsplatten von 3-6 mm.

7. Elastischer verstärkter Zement-Verbundwerkstoff nach Anspruch 1, ferner **gekennzeichnet durch**:
(a) Verwenden eines perforierten röhrenförmigen Kragen-Hülsen-Verbindungsstücks mit einer räumlichen Struktur von dreieckigem Querschnitt für Spleißverbindungen zwischen zwei koaxialen perforierten röhrenförmigen Bewehrungen mit gleichen Außenabmessungen;
(b) Verwenden eines gebogenen/mehrfach verzweigten Kragen-Hülsen-Verbindungsstücks zum Ausrichten/Orientieren mehrerer Spleißverbindungen aus einer Vielzahl von perforierten röhrenförmigen Bewehrungen;
(c) Innenabmessungen des perforierten röhrenförmigen Kragen-Hülsen-Verbindungsstücks, die gleich Außenabmessungen der beiden koaxialen perforierten röhrenförmigen Bewehrungsstäben sind, sodass eine passgenaue Einsteckverbindung zuverlässig ausgebildet werden;
(d) eine integrierte Form eines Kontakt-Läpp- und Spleißhülse-Mechanismus, um eine kontinuierliche Kraftübertragung zwischen den durchgehenden massiven Scheitelecken der perforierten röhrenförmigen Kragenhülse und den koaxialen perforierten röhrenförmigen Bewehrungsstäben herzustellen; und
(e) Verwenden eines Dübelverankerungsmechanismus mit infiltrierter Zementmatrix für die Verflechtung von perforierten röhrenförmigen Kragenhülsen und koaxialen perforierten röhrenförmigen Bewehrungsstäben.

8. Elastischer verstärkter Zement-Verbundwerkstoff nach Anspruch 1, ferner **gekennzeichnet durch**:
(a) Verwenden eines Warmstrangpressprozesses für Metallrohre, um hohe Längsdehnungsfähigkeitseigenschaften zu erzielen;
(b) Verwenden eines Faserlaser-Herstellungsprozesses, um hochgenaue Maßeigenschaften der Perforation in Verbindung mit einem minimalen Wärmezoneneffekt (HAE) zu definieren; und
(c) Verwenden eines Faserlaser-Ätzprozesses, der zu einer aufgerauten Oberflächentextur der Bewehrungsstab-Struktur führt, um Bindungseigenschaften zu verbessern.

9. Elastischer verstärkter Zement-Verbundwerkstoff nach Anspruch 1, ferner **dadurch gekennzeichnet, dass** er zur Verwendung als Strukturkomponenten und/oder -elemente beim Ausbilden von vor Ort und/oder vorgefertigten verstärkten Zement-Verbundwerkstoffkomponenten bestimmt ist und Folgendes aufweist:
(a) eine hohe Querschnittsduktilität für sowohl axial als auch horizontal belastete Komponenten, die durch die hochsteife verteilte Ringzugwirkung der periodisch angeordneten perforierten Quermetallplatte als der Dehnung entgegenwirkende Innenbewehrung bewirkt wird;
(b) hohe Verformungsfähigkeit für die axial und/oder horizontal belasteten strukturellen Komponenten, die durch die dreidimensional gestaltete zellenförmige Bewehrungsstabeinschließungs-Käfigstruktur bewirkt wird, wodurch in dem verstärkten Zement-Verbundwerkstoff eine einzigartige und effektive, verteilte, ineinandergreifende Dübelzelleneinheit bereitgestellt wird; und
(c) hohes seismisches Reaktionsvermögen für Balken-Rahmen-Strukturkomponenten, die durch die Kernzonen-Ringspannungsbewehrung des selbststehenden Netzwerks aus dreieckigen Bewehrungsstäben bewirkt wird, indem sie kontinuierlich Widerstand gegen diagonale Spannung aufgrund von Scherung leistet.

10. Elastischer verstärkter Zement-Verbundwerkstoff nach Anspruch 9, ferner **dadurch gekennzeichnet, dass** die vorgefertigten, bewehrten Zement-Verbundwerkstoff-Komponenten ein System aus Stützen, Balken und Balken-Rahmen für die Errichtung von Gebäuden und zivilen Strukturen einschließen.

11. Elastischer verstärkter Zement-Verbundwerkstoff nach Anspruch 2, ferner **dadurch gekennzeichnet, dass** die perforierten, Platten (E) mit einem Muster aus dreieckigen Löchern aus einem bearbeiteten Feinkornmaterial sind, das Folgendes aufweist:
(a) das perforierte Metallblech, das durch warmgewalztes dünnes Metall mit niedrigem Kohlenstoffgehalt mit einer hohen Zugfestigkeit von mindestens 250 MPa und einer hohen Längsdehnbarkeit von mindestens 20% ausgebildet wird;
(b) den konstruierten Ring mit dreieckiger Geometrie, vorzugsweise mit einer gleichseitigen Form, um das Netzwerk aus periodischen Gitterrippen und Knoten auszubilden, das nahezu isotrope Eigenschaften und verteilte endlose Ring-Einschließungselemente aufweist;
(c) den konstruierten Ring mit einer Längsabmessung zwischen 30 mm und 70 mm, mit einem verschwimmenden und/oder nicht verschwimmenden Rand;
(d) die hochsteife, feinkörnige Matrix-Lochplatten-Bewehrungsphase mit einer Plattendicke zwischen 2 mm und 5 mm und einem Stapelabstand zwischen 30 mm und 100 mm, was mindestens 2,5-mal so groß ist wie die maximale Aggregat-Korngröße der infiltrierten Matrixphase;
(e) den befreiten Steg mit einer Dicke-Abmessung zwischen 5 mm und 20 mm;
(f) die Ringe mit endlosem Dreiecksmotiv der Lochgitterplatte mit einem optimalen Formfaktorverhältnis zwischen der Gesamtumfangslänge des Rings und der maximalen Aggregat-Korngröße der Matrixphase, der mindestens größer als 10 ist; und
(g) die Ringe mit endlosem Dreiecksmotiv der Lochgitterplatte mit einer Ringgröße, die mindestens 2,5-mal so groß ist wie die maximale Aggregat-Korngröße der infiltrierten Matrixphase.

12. Elastischer verstärkter Zement-Verbundwerkstoff nach Anspruch 11, ferner **dadurch gekennzeichnet, dass** der konstruierte Ring in Längsrichtung eine Abmessung zwischen 40 mm und 60 mm aufweist mit einem nicht-verschwimmenden und/oder verschwimmenden Rand.

13. Elastischer verstärkter Zement-Verbundwerkstoff nach Anspruch 11, ferner **dadurch gekennzeichnet, dass** die hochsteife Feinkornmatrix-Lochplatten-Bewehrungsphase einen Stapelabstand zwischen 40 mm und 60 mm aufweist.

14. Elastischer verstärkter Zement-Verbundwerkstoff nach Anspruch 11, ferner **dadurch gekennzeichnet, dass** der befreite Steg eine Dicke zwischen 5 mm und 15 mm aufweist.

15. Elastischer verstärkter Zement-Verbundwerkstoff nach Anspruch 11, ferner **dadurch gekennzeichnet, dass** die Ringe mit endlosem Dreiecksmotiv der Lochgitterplatte ein optimales Formfaktorverhältnis zwischen der Gesamtumfangslänge des Rings und der maximalen Aggregat-Korngröße der Matrixphase von mindestens größer als 20 aufweisen.

16. Elastischer verstärkter Zement-Verbundwerkstoff nach Anspruch 2, ferner **dadurch gekennzeichnet, dass** die monolithische, dreidimensional verstärkte VerbundwerkstoffStruktur eine Sandwich-Raumstruktur einer Vielzahl von plattenförmigen Matrizen mit hoher Steifigkeit ist, in denen in der ersten, zweiten und dritten Dimension langgestreckte Bewehrungskomponenten mit minimaler Masse eingebettet sind, und zwar mit:
(a) dem hohen Widerstand gegen Abplatzen beim Biegen mit einer größeren aktiven Verbindungszone, und zwar durch Anwenden einer Sandwich-Raumstruktur als dünne Platten, welche zu Bündeln zusammengebaut sind, die Verbundplatten ausbilden, was einem größeren Trägheitsmoment entspricht;
(b) der Beschränkung der minimierten Steifigkeitsfehlanpassung zwischen der Bewehrungs- und der Matrixphase; und
(c) der Beseitigung von Schweißen und/oder Klebematerial im Inneren des Verbundwerkstoffs, um dadurch eine kompakte, ermüdungsbeständige Struktur zu verwirklichen.

17. Elastischer verstärkter Zement-Verbundwerkstoff nach Anspruch 2 zur Verwendung als Strukturelement oder Komponente, ferner **dadurch gekennzeichnet, dass** er Folgendes umfasst:
(a) mehrschichtige perforierte Metallgitterplattenelemente (E) zum Ineinandergreifen (b);
(b) eine Vielzahl von perforierten, hohlen, röhrenförmigen Metallbewehrungskörpern (F) als Verbindungsstücke und Abstandshalter, die (c) erzeugen;
(c) durchgehende Bewehrungsstrukturphase (B) aus ineinandergreifenden dreidimensionalen Gitterzellen und versteift durch (d);
(d) Infiltration von anorganischem Zementmatrix-Hochleistungsbindemittel (A), und, nach dem Aushärten, synergistisches Ausbilden von (e); und
(e) vollständig steife, dünne, ein- oder mehrschichtige, strukturierte, monolithische, laminatförmige Sandwich-Verbundwerkstoff-Strukturkomponente oder -element mit einem hohen Verhältnis von Eigenfestigkeit zu Gewicht für allgemeine und spezielle Anwendungen im Bauwesen und in anderen Industrien.

18. Elastischer verstärkter Zement-Verbundwerkstoff nach Anspruch 2, ferner **dadurch gekennzeichnet, dass** er eine Hybridisierungsstrategie für strukturierte Strukturen aus mehreren Materialien mit vorbestimmten geometrischen Konfigurationen aufweist, einschließlich zellenförmig, schicht- und röhrenförmig konfigurierter Strukturen, um Phasen aus geordnetem Material zu bilden, um einen ein- und/oder mehrschichtigen Sandwich-Verbundwerkstoff auszubilden mit:
(a) hoher Druck- und Zugfestigkeit, hoher Steifigkeit;
(b) hoher globaler Duktilität und Verformungsfähigkeit; und
(c) hoher Toleranz gegenüber lokalen mechanischen Beschädigungen.

19. Elastischer verstärkter Zement-Verbundwerkstoff nach Anspruch 2, ferner **dadurch gekennzeichnet, dass** die monolithische, dreidimensional verstärkte VerbundwerkstoffStruktur eine Sandwich-Raumstruktur ist aus einer Vielzahl von plattenförmigen Matrizen mit hoher Steifigkeit umfasst, in die langgestreckte an den Scheiteln angeordneten miteinander verbundene massive dreieckige perforierte hohlen Bewehrungskomponenten in der ersten, zweiten und dritten Dimension mit minimaler Masse eingebettet sind, und zwar mit:
(a) dem hohen Widerstand gegen Abplatzen beim Biegen mit einer größeren aktiven Verbindungszone, und zwar durch Anwenden der Sandwich-Raumstruktur als dünne Platten, welche zu Bündeln zusammengebaut sind, Verbundplatten ausbilden, was einem größeren Trägheitsmoment entspricht;
(b) der Beschränkung der minimierten Steifigkeitsfehlanpassung zwischen der Bewehrungs- und der Matrixphase; und
(c) Beseitigung von Schweißen und/oder Klebematerial im Inneren des Verbundwerkstoffs, um dadurch eine kompakte, ermüdungsbeständige Struktur zu verwirklichen.

20. Elastischer verstärkter Zement-Verbundwerkstoff nach Anspruch 6, ferner **dadurch gekennzeichnet, dass** er minimiert wird, indem er eine direkte Überlappung von Einschließungsringen zur Kraftübertragung in angrenzenden Platten aufweist.

21. Elastischer verstärkter Zement-Verbundwerkstoff nach Anspruch 11 zur Verwendung als Strukturkomponenten oder -elemente bei der Herstellung modularer Komponenten für die Anwendung eines Verfahrens der Baugruppenbauweise während des Betriebs vor Ort.

22. Elastischer verstärkter Zement-Verbundwerkstoff nach Anspruch 21, ferner **dadurch gekennzeichnet, dass** die genannten Strukturkomponenten oder -elemente aus einschichtigen, strukturierten, zellenförmigen Laminat-Wandpaneelen und Plattenpaneelen zusammengebaut sind, die nach dem gegenseitigen Zusammenbauen der modularen Komponenten an Ort und Stelle und anschließender Infiltration der Matrix (A) vor Ort eine Vielzahl der elastischen verstärkten zementhaltigen Verbundwerkstoffe nach Anspruch 2 ausbilden.

23. Wohngebäude, das aus Strukturkomponenten oder -elementen zusammengesetzt ist, wobei die Strukturkomponenten aus dem elastischen verstärkten Zement-Verbundwerkstoff nach Anspruch 21 und einer Vielzahl der elastischen verstärkten Zement-Verbundwerkstoffe nach Anspruch 2 bestehen.

## Revendications

1. Nouveau composite cimentaire renforcé élastique (10) qui est constitué d'une barre de renforcement en matériau métallique tubulaire perforée sans soudures monolithique allongée avec une topologie de confinement de section triangulaire configurée par trois parties en forme de tige solides, interconnectées, alignées, parallèles et continues situées au niveau de sommets triangulaires (21) respectivement en tant que phase de renforcement longitudinale, plusieurs parties formant pansement à coque à mi-longueur perforées en tant que phase d'ancrage, et un matériau liant hydraulique à module élastique élevé, à mélange hétérogène infiltré en tant que phase matricielle, dans lequel un réseau de goujons d'ancrage à liaison mécanique répartie, à alignment axial, radiaux par rapport au noyau et uniques, effectué à partir de cellules unitaires (42) de goujons à matrice multicellulaire, formé de manière synergique de manière unitaire avec des cercles (31) de confinement cellulaire sans fin le long de la coque perforée à mi-longueur pendant la solidification du composite du liant hydraulique ;
la nouvelle barre de renforcement tubulaire perforée (20) étant un matériau métallique extrudé de forme fermée ayant une topologie de section triangulaire équilatérale pour maximiser le moment d'inertie de ladite structure de barre de renforcement ;
les coins de sommet solides continus allongés (21) de la barre de renforcement de topologie de section triangulaire équilatérale étant désignés phases de renforcement pour maximiser la rigidité de ladite structure de barre de renforcement ;
la partie formant pansement à coque à mi-longueur perforée (22) de la topologie de section triangulaire équilatérale étant désignée phase d'ancrage avec les cercles (31) de confinement cellulaire sans fin agencés périodiquement pour maximiser l'action de verrouillage et de confinement de ladite structure de barre de renforcement sur des goujons de matrice ;
les coins de sommet solides continus allongés (21) étant connectés de manière monolithique par les parties à coque à mi-longueur perforées (22) de ladite barre de renforcement pour maximiser l'action de liaison composite avec la matrice infiltrée, éliminant ainsi l'effet de décalage de cisaillement d'une structure de barre de renforcement solide épaisse traditionnelle ;
les coins de sommet solides continus allongés (21) étant connectés de manière monolithique par les parties de pansement à coque à mi-longueur perforées pour maximiser la capacité anti-flambage de ladite structure de barre de renforcement ;
les têtes de capuchons d'extrémité d'ancrage en forme de profil (24) maximisant la capacité d'ancrage et raccourcissant l'exigence de longueur d'encastrement de ladite structure de barre de renforcement ;
le matériau de matrice (40) de liant hydraulique à mélange ternaire à module élastique élevé infiltré renforçant la capacité anti-flambage de ladite structure de barre de renforcement ;
la nouvelle barre de renforcement tubulaire perforée de forme triangulaire étant conçue avec un réseau de cellules unitaires de goujons de confinement multicellulaires (42) en tant que mécanisme de liaison principal de verrouillage d'interfaces de matrices de ladite structure de barre d'armature de renforcement ; et
les nouvelles barres de renforcement tubulaires perforées de forme triangulaire étant assemblées longitudinalement pour former un réseau de barres de renforcement triangulaires à l'état autonome par couplage avec une pluralité de plaques métalliques multicouches (30) ayant des trous de réception perforés de forme triangulaire configurés en tant que système de cercles de confinement de renforcement latéral.

2. Composite cimentaire renforcé élastique selon la revendication 1, **caractérisé en outre en ce que** :
il a une topologie stratifiée ;
au moins un domaine dudit composite cimentaire renforcé élastique a une structure de composite renforcée en trois dimensions comprenant une matrice cimentaire à base de laitier de haut fourneau granulé très fin partitionnée (A) avec une structure de réseau de barre d'armature creuse cellulaire verrouillée en tension (B) intégralement incorporée dans la matrice (A), le système de matrice (A) comprenant une phase (C) d'une pluralité de d'unités de goujons à inclusion dure cellulaires, cylindriques, triangulaires formées in situ, et phase (D) d'une pluralité d'unités souples, cellulaires, hexagonales, répliquées, le réseau de barres d'armature verrouillées en tension (B) comprenant des plaques (E) à motifs de trous triangulaires perforées multicouches empilées en parallèle et verrouillées en tension par une pluralité de corps de barres d'armature (F) creux triangulaires perforés solides de sommet dans la direction transversale ;
il conçoit la dimension, l'alignement et la densité des composants de renforcement verrouillés en tension de forme triangulaire pour un réglage de la résistance ;
il conçoit le volume, l'épaisseur et l'espacement de couches des plaques métalliques perforées à motifs de nervures d'iso-grille empilées en parallèles pour un réglage d'une résistance à la compression, une rigidité et d'une ductilité ; et
il conçoit la topologie de confinement du réseau de goujons de matrice d'ancrage formés in situ pour un réglage d'une résistance au cisaillement.

3. Composite cimentaire renforcé élastique selon la revendication 1, caractérisé en outre :
(a) en ce qu'il inclut un « module CEM » ayant un matériau de matrice « germe G » de liant hydraulique à module élastique élevé réglable à mélange hétérogène infiltré ;
(b) ledit matériau de matrice de liant hydraulique à mélange ternaire comprenant du ciment de Portland (OPC), un laitier de haut fourneau granulé (GGBS) et un laitier de haut fourneau granulé très fin (UFGGBS) en association avec un codispersant polymère en tant qu'espaceur osmotique pour former de manière synergique un matériau de matrice frais avec des propriétés rhéologiques de faible limite d'écoulement et de faible viscosité tout en, après durcissement, possédant des propriétés mécaniques de module élastique élevé dérivées d'une densité de conditionnement à liaison optimisée dudit liant ternaire ;
c) ledit matériau de matrice de liant hydraulique à mélange ternaire comprenant un agent codispersant hautement efficace pour améliorer l'aptitude de remplissage de charge minérale active ultrafine du liant et une densité de conditionnement global optimisée avec une épaisseur eau-film moindre ;
(d) ledit matériau de matrice de liant hydraulique à mélange ternaire ayant une composition au niveau de la meilleure performance agencée dans une proportion telle que OPC-30 µm (50-60 %), GGBS-20 µm (10-25 %), UFGGBS-10 µm~5 µm (15-35 %) en poids de la teneur de liant totale ;
(e) ledit matériau de matrice de liant hydraulique à mélange ternaire avec un rapport eau-liant pour la meilleure performance attribué de 0,30-0,33 pour obtenir une aptitude à l'autocompactage pendant un stade de coulée avec une gamme de débits entre 650 mm et 800 mm en ajustant le dosage d'agent de fluidisation ;
(f) ledit matériau de matrice de liant hydraulique à mélange ternaire ayant un rapport liant-agrégat au niveau de la meilleure performance désigné comme 0,30-0,33 pour obtenir une densité de conditionnement global élevée ; et
(g) ledit matériau de matrice de liant hydraulique à mélange ternaire au niveau de la meilleure performance après un durcissement complet à 28 jours ayant un module d'élasticité dans la plage de 35-45 GPa, et une résistance à la compression dans la plage de 60-80 MPa.

4. Composite cimentaire renforcé élastique selon la revendication 3, **caractérisé en outre en ce que** le matériau de matrice de liant hydraulique à mélange ternaire au niveau de la meilleure performance après un durcissement complet à 28 jours a un module d'élasticité dans la plage de 40-45 GPa.

5. Composite cimentaire renforcé élastique selon la revendication 1, **caractérisé en outre en ce que** la barre de renforcement de matériau métallique tubulaire perforée sans soudures monolithique avec une topologie de section triangulaire inclut :
(a) une capacité anti-flambage élevée développée à partir de l'action restreignante du noeud de pansement en cercle triangulaire fermé espacé périodiquement de la barre de renforcement tubulaire ;
(b) une résistance à la liaison anti-dérapante élevée par le biais d'une action verrouillante de goujons de confinement entre la barre de renforcement et la matrice de béton ;
(c) une résistance à l'ancrage mécanique élevée par le biais d'un capuchon à profil droit et/ou en L pour raccourcir la longueur de développement d'intégration ;
(d) des cercles cellulaires sans fin à forte capacité de confinement configurés par une épaisseur de coque à mi-longueur perforée d'au moins 3-6 mm, une taille de trou perforé d'au moins 25-40 mm et une largeur de barre de réticulation d'au moins 6-12 mm ;
(e) une résistance à la défaillance élevée avec un diamètre de section de tige solide interconnectée au sommet dans la plage de 8-25 mm ;
(f) une résistance élevée à l'allongement de l'acier dans la plage de la qualité d'acier 275-500 ; et
(g) une ductilité et une capacité à la déformation élevées avec un pourcentage d'allongement d'au moins 20-30 %.

6. Composite cimentaire renforcé élastique selon la revendication 1, **caractérisé en ce qu'**il a un réseau de barres de renforcement triangulaires à l'état autonome avec :
(a) une action restreignant le support latéral hautement efficace effectuée par l'action de matage verrouillé entre une pluralité de plaques de renforcement transversales perforées espacées périodiquement et une pluralité de barres de renforcement métalliques tubulaires longitudinales perforées allongées ;
(b) des plaques de renforcement transversales perforées ayant une rigidité élevée au cisaillement avec une configuration de déchets d'isogrille et des trous triangulaires équilatéraux pour l'insertion par couplage des barres de renforcement métalliques tubulaires perforées ; et
(c) une résistance élevée à la défaillance avec une épaisseur de plaques de renforcement latérales perforées dans la plage de 3-6 mm.

7. Composite cimentaire renforcé élastique selon la revendication 1, **caractérisé en outre par** :
(a) l'utilisation d'un connecteur collier-manchon tubulaire perforé de topologie de section triangulaire pour des connexions d'épissure entre deux barres d'armature tubulaires perforées coaxiales de mêmes dimensions extérieures ;
(b) l'utilisation d'un connecteur collier-manchon façonné courbé/à ramifications multiples pour aligner/orienter plusieurs articulations de connexion d'épissure parmi une pluralité de barres d'armature tubulaires perforées ;
(c) le fait qu'il présente des dimensions internes de connecteur collier-manchon tubulaire perforé égales à des dimensions extérieures des deux barres d'armature tubulaires perforées coaxiales de telle sorte que des connexions d'insertion étroites sont formées de manière fiable ;
(d) le fait qu'il présente une forme intégrale de mécanisme de rodage de contact et de manchon d'épissure pour établir un transfert de forces continu entre les coins de sommet solides continus du manchon de collier tubulaire perforé et les barres d'armature tubulaires perforées coaxiales ; et
(e) l'utilisation d'un mécanisme d'ancrage de goujons à matrice cimentaire infiltrés pour verrouiller un manchon-collier tubulaire perforé et des barres d'armature tubulaires perforées coaxiales.

8. Composite cimentaire renforcé élastique selon la revendication 1, **caractérisé en outre par** :
(a) l'utilisation d'un processus de formage de tube métallique par extrusion à chaud pour obtenir des propriétés d'allongement à la traction élevées ;
(b) l'utilisation d'un processus de fabrication laser à fibres pour définir des propriétés de dimensions de perforations de haute précision associées à un effet de zone de chaleur minimum (HAE) ; et
(c) l'utilisation d'un processus de gravure laser sur fibres se traduisant par une texture de surface de structure de barre d'armature rugueuse pour améliorer des caractéristiques de liaison.

9. Composite cimentaire renforcé élastique selon la revendication 1, **caractérisé en outre en ce qu'**il est destiné à une utilisation en tant que composants et/ou éléments structuraux dans la formation de composants composites cimentaires renforcés in situ et/ou préfabriqués, et ayant :
(a) une performance de ductilité de section élevée pour des composants structuraux à charge axiale et/ou horizontale effectuée par l'action de tension de cercles distribués à rigidité élevée de la plaque métallique transversale perforée espacée périodiquement en tant que renforcement interne anti-dilatation ;
(b) une capacité élevée à la déformation pour les composants structuraux à charge axiale et/ou horizontale effectuée par la structure de cage de confinement à barres d'armature cellulaire conçue de manière tridimensionnelle, fournissant ainsi des unités cellulaires de goujons de verrouillage distribuées uniques et efficaces dans le composite cimentaire renforcé ; et
(c) une performance élevée de réponse sismique pour des composants structuraux de poutre-châssis effectuée par le renforcement en tension de cercles de zone centrale du réseau de barres de renforcement triangulaires à l'état indépendant en fournissant une résistance à la tension en diagonale en raison du cisaillement de manière continue.

10. Composite cimentaire renforcé élastique selon la revendication 9, **caractérisé en outre en ce que** lesdits composants de composite cimentaire renforcé préfabriqués incluent un système de colonnes, poutres et poutre-colonne pour l'érection de bâtiments et de structures civiles.

11. Composite cimentaire renforcé élastique selon la revendication 2, caractérisé en ce outre en ce que les plaques à motifs (E) à trous triangulaires perforées sont un matériau à grain fin conçu présentant :
(a) la plaque métallique perforée formée par un métal fin bas carbone laminé à chaud avec une résistance élevée à la traction qui est d'au moins 250 MPa et une ductilité élevée à allongement qui est d'au moins 20 % ;
(b) le cercle de confinement avec une géométrie en triangle, de préférence une forme équilatérale pour former la toile périodique de nervures et de noeuds de grille ayant une propriété presque isotrope et des éléments de confinement de cercle sans fin distribués ;
(c) le cercle conçu avec une dimension longitudinale entre 30 mm et 70 mm avec une bordure de non-floutage et ou une bordure de floutage ;
(d) la phase de renforcement de plaques perforées à matrice à grain fin à rigidité élevée avec une épaisseur de plaque entre 2 mm et 5 mm et un espacement d'empilement entre 30 mm et 100 mm, qui représente au moins 2,5 fois la dimension de la granulométrie d'agrégat maximale de la phase matricielle d'infiltration ;
(e) la toile débarrassée avec une dimension en épaisseur entre 5 mm et 20 mm ;
(f) les cercles des motifs en triangle sans fin de la plaque de grille perforée ayant un rapport de facteur de forme optimum entre la longueur de périmètre totale du cercle et la granulométrie d'agrégat maximum de la phase matricielle au moins supérieure à 10 ; et
(g) les cercles des motifs en triangle sans fin de la plaque de grille perforée ayant une taille de cercle qui représente au moins 2,5 fois la dimension de la granulométrie d'agrégat maximum de la phase matricielle d'infiltration.

12. Composite cimentaire renforcé élastique selon la revendication 11, **caractérisé en outre en ce que** le cercle conçu a une dimension longitudinale entre 40 mm et 60 mm avec une bordure de non-floutage et ou une bordure de floutage.

13. Composite cimentaire renforcé élastique selon la revendication 11, **caractérisé en outre en ce que** la phase de renforcement de plaques perforées à matrice de grains fins de rigidité élevée présente un espacement d'empilement entre 40 mm et 60 mm.

14. Composite cimentaire renforcé élastique selon la revendication 11, **caractérisé en outre en ce que** le ruban débarrassé a une dimension en épaisseur entre 5 mm et 15 mm.

15. Composite cimentaire renforcé élastique selon la revendication 11, **caractérisé en outre en ce que** les cercles à motifs en triangle sans fin de la plaque de grille perforée ont un rapport de facteurs de forme optimum entre la longueur totale de périmètre du cercle et une granulométrie d'agrégat maximum de la phase matricielle au moins supérieure à 20.

16. Composite cimentaire renforcé élastique selon la revendication 2, **caractérisé en outre en ce que** la structure de composite renforcée en trois dimensions monolithique est un groupement à topologie en sandwich d'une pluralité de matrices en forme de plaque à rigidité élevée dans lesquelles sont intégrés des composants de renforcement allongés dans les première, deuxième et troisième dimensions avec une masse minimum avec :
(a) la résistance élevée au pelage lors d'un cintrage avec une zone de connexion active plus grande en employant une topologie en sandwich en tant que panneaux fins assemblés en faisceaux formant des panneaux composites, ce qui correspond à un moment d'inertie plus grand ;
(b) la limitation de décalage de rigidité minimisé entre les phases de renforcement et matricielles ; et
(c) l'élimination du matériau de soudage ou adhésif à l'intérieur du composite pour ainsi réaliser une structure compacte résistante à la fatigue.

17. Composite cimentaire renforcé élastique selon la revendication 2 destiné à une utilisation en tant qu'élément ou composant structural, **caractérisé en outre en ce qu'**il comprend :
(a) des éléments de plaque de grille perforés en métal à plusieurs couches (E) pour un verrouillage (b) ;
(b) une pluralité de corps de renforcement (F) tubulaires, métalliques, creux, perforés en tant que connecteurs et espaceurs générant (c) ;
(c) une phase de structure à renforcement continu (B) à cellules de grille en trois dimensions d'inter-verrouillage et raidies par (d) ;
(d) une infiltration de matériau de liant (A) à matrice cimentaire inorganique haute performance et, après durcissement, la formation de manière synergique de (e) ; et
(e) un composant ou élément structurel composite structuré en sandwich stratifié monolithique conçu de manière monocouche ou multicouche mince complètement rigide avec un rapport résistance intrinsèque sur rapport pondéral élevé pour des applications générales et spécialisées dans la construction et d'autres industries.

18. Composite cimentaire renforcé élastique selon la revendication 2, **caractérisé en outre en ce qu'**il a une stratégie d'hybridation de structures structurées avec des matériaux multiples avec des configurations topologiques prédéterminées incluant des structures à configuration cellulaire, en couche et tubulaire pour constituer des phases de matériau ordonnées pour former un composite en sandwich monocouche et ou multicouche avec :
(a) une résistance élevée à la compression et à la traction, une rigidité élevée ;
(b) une ductilité globale et une capacité de déformation élevées ; et
(c) une tolérance élevée des dommages mécaniques locaux.

19. Composite cimentaire renforcé élastique selon la revendication 2, **caractérisé en outre en ce que** la structure de composite renforcée en trois dimensions monolithique est un groupement de topologies en sandwich d'une pluralité de matrices en forme de plaque à rigidité élevée dans lesquelles sont intégrés des composants de renforcement creux, triangulaires, perforés, solides, de sommet, allongés, dans des première, deuxième et troisième dimensions avec une masse minimum avec :
(a) la résistance élevée au pelage lors d'un cintrage avec une zone de connexion active plus grande en employant la topologie en sandwich en tant que panneaux fins assemblés en faisceaux formant des panneaux composites ce qui correspond à un moment d'inertie plus grand ;
(b) la limitation de décalage de rigidité minimisé entre les phases de renforcement et matricielles ; et
(c) l'élimination du matériau de soudage et ou adhésif à l'intérieur du composite pour ainsi réaliser une structure compacte résistante à la fatigue.

20. Composite cimentaire renforcé élastique selon la revendication 6, **caractérisé en outre en ce qu'**il est minimisé en ayant un chevauchement direct de cercles de confinement pour transférer de la force dans des plaques adjacentes.

21. Composite cimentaire renforcé élastique selon la revendication 11 destiné à une utilisation en tant que composants ou éléments structuraux dans la fabrication de composants modulaires pour l'adoption d'un procédé de construction de type assemblage pendant le fonctionnement sur site.

22. Composite cimentaire renforcé élastique selon la revendication 21, **caractérisé en outre en ce que** lesdits composants ou éléments structuraux sont composés de panneaux de paroi stratifiés cellulaires et de panneaux de dalles conçus de manière monocouche, qui, après assemblage réciproque desdits composants modulaires *in situ,* suivi par une infiltration *in situ* de la matrice (A) forment une pluralité du composite cimentaire renforcé élastique selon la revendication 2.

23. Bâtiment pour habitation composé de composants ou éléments structuraux, dans lequel lesdits composants structuraux sont composés du composite cimentaire renforcé élastique selon la revendication 21 et d'une pluralité du composite cimentaire renforcé élastique selon la revendication 2.
